

Patented Jan. 31, 1928.

## UNITED STATES PATENT OFFICE.

CHARLES SAMUEL BEDFORD, OF LEEDS, ENGLAND.

## DYEING ARTIFICIAL SILK.

No Drawing. Application filed August 31, 1926, Serial No. 132,899, and in Great Britain September 21, 1925.

This invention relates to the dyeing of artificial silk and has for its object an improved method of dyeing such silk.

By artificial silk I mean the various fibres now upon the market, consisting of cellulose rendered viscous by the acetyl, xanthate or similar process and extruded through spinnerets of suitable diameter to form silk-like filaments of any desired grade or "denier".

Up to the present it has not been practicable to dye this material black by means of logwood owing to the fact that chromium oxide, the use of which is inherent to dyeing with logwood, exhibits little affinity for the fibre.

According to this invention I have found that such fibres have the remarkable property of absorbing logwood colouring matter from an aqueous solution which can be neutral, acid or alkaline, thereby becoming light orange to dark brown in colour. The logwood liquor may be used cold or hot. Viscose and similar fibres develop to a good black after treatment with logwood dye in the cold, but acetyl silk such as celanese requires to be steeped hot. When the silk so treated is placed in a hot bath of sodium bichromate, chromium oxide is fixed and an intense black is obtained.

After washing hot and a light scouring in soap, the shades are fast to boiling, soap and milling.

The following examples, which are by no means limitative, describe a particular manner of carrying out my invention in the case of cellulose acetate (celanese) silk.

*Example 1.*—Cellulose acetate celanese silk, yarn or fabric is steeped in a bath consisting of a solution of from 2 to 5% logwood crystals or hematine.

The silk is treated in this manner at a temperature of from 60° to 100° C. preferably at 70 to 80° C. for 15 to 30 minutes. It is then taken out and washed in water, or pressed through rollers, or whizzed, and immediately passed into a bath containing a 1 to 3% solution of sodium bichromate at a temperature not less than 60° C. The black begins to develop at once and the dyeing is completed in 10 to 30 minutes, or the silk may be passed into a cold chrome bath and gradually heated up to 80° C.

The chrome bath may be used without any other addition whatever, but it is advisable especially when acid has been used

with the logwood dye to add a little chalk or mild alkali, such as sodium carbonate or bi-carbonate, sodium acetate, ammonium carbonate, or borax; this causes the black formed to be a bluer shade.

Both the logwood and the chrome baths can be used for dyeing successive lots of silk, but they require strengthening by further additions of hematine and sodium bichromate. Finally by addition of about 5% of common salt or of Glauber's salt without further addition of water they may be economically exhausted.

In other cases I steep silk in a 2 to 5% solution of logwood crystals or hematine, alone or with addition of 5% (on the water) Turkey red oil. After steeping for 10 to 30 minutes the fibre is taken out, rolled or whizzed, and dried. The black is developed in a hot solution of sodium bichromate as above described.

It is obvious that the process is equally suited for dyeing piece goods as well as yarn, also for goods consisting in part of wool or natural silk.

*Example 2.*—Viscose silk is treated exactly as described in Example 1, but the temperature of the logwood bath may range from 20° to 93° C. The temperature of the chrome in the case of viscose may be varied from 20° to 93° C. I am of opinion however that faster shades are given by using a hot chrome bath.

*Example 3.*—When treating a fabric consisting of a mixture of cellulose acetate (celanese) and viscose artificial silk, if, for any reason, it is desirable to leave the cellulose acetate celanese silk undyed, the fabric after treatment with logwood dye in the cold is developed in cold sodium bichromate solution (from 1 to 3%). By this means black is developed on the viscose silk but the celanese silk remains undyed. The celanese silk can afterwards be dyed up with suitable colours to produce mixed colour effects.

On the other hand, although the various kinds of artificial silk exhibit a selective action towards dyestuffs, so that it is almost impossible to dye a piece containing two or more kinds of fibre, by the usual processes, to the same shade of black, this desirable result can be obtained by my process when carried out as before described in Example 1.

What I claim and desire to secure by Letters Patent is:—

1. The process of dyeing yarns and fabrics comprising artificial silk, consisting in first 5 impregnating the fibre with logwood dye, and subsequently developing in a solution of alkali bichromate.
  2. The process of dyeing yarns and fabrics comprising artificial silk, consisting in first 10 impregnating the fibre with logwood dye, and subsequently developing in a solution of sodium bichromate.
  3. The process of dyeing yarns and fabrics constituted by a mixture of cellulose acetate 15 and viscose silks, consisting in impregnating the fibres with logwood dye and afterwards developing in alkali bichromate solution.
  4. The process of dyeing yarns and fabrics constituted by a mixture of cellulose acetate 20 and viscose silks, consisting in impregnating the fibres with logwood dye and afterwards developing in sodium bichromate solution.
  5. The process of dyeing yarns and fabrics comprising artificial silk, consisting in first 25 impregnating the fibre with logwood dye, and subsequently developing a black by steeping in a solution of alkali bichromate at a temperature of from 60° to 100° C.
  6. The process of dyeing yarns and fabrics comprising artificial silk, consisting in first 30 impregnating the fibre with logwood dye, and subsequently developing a black by steeping in a solution of alkali bichromate at a temperature of from 60° to 100° C. to which has been added a mild alkali.
  7. The process of dyeing yarns and fabrics comprising artificial silk, consisting in first 35 impregnating the fibre with logwood dye,
- and subsequently developing a black by steeping in a solution of alkali bichromate <sup>40</sup> at a temperature of from 60° to 100° C. to which has been added borax.
8. The process of dyeing yarns and fabrics comprising artificial silk, consisting in first impregnating the fibre with logwood dye, <sup>45</sup> and subsequently developing a black by steeping in a solution of sodium bichromate at a temperature of from 60° to 100° C.
  9. The process of dyeing yarns and fabrics comprising artificial silk, consisting in first <sup>50</sup> impregnating the fibre with logwood dye to which Turkey red oil has been added, and subsequently developing a black by steeping in a solution of sodium bichromate at a temperature of from 60° to 100° C. <sup>55</sup>
  10. Yarns and fabrics comprising artificial silk dyed by impregnating with logwood dye and subsequently developing in a solution of alkali bichromate.
  11. Yarns and fabrics comprising artificial silk constituted by a mixture of cellulose acetate and viscose silks, dyed by impregnating the fibres with logwood dye and afterwards developing in alkali bichromate solution. <sup>60</sup>
  12. The process of dyeing yarns and fabrics comprising artificial silk, consisting in first impregnating the fibre with logwood dye, and subsequently developing a black by steeping in a solution of alkali bichromate at a temperature of from 60° to <sup>70</sup> 100° C. to which has been added sodium acetate. <sup>65</sup>

In testimony whereof I affix my signature.

CHARLES SAMUEL BEDFORD.